

## UNITED STATES PATENT OFFICE

2,027,389

## PACKING FLUID SEALS

Wilbur Arthur Lazier, Wilmington, Del., assignor  
to E. I. du Pont de Nemours & Company, Wil-  
mington, Del., a corporation of Delaware

No Drawing. Application June 19, 1931.  
Serial No. 545,487

## 10 Claims. (Cl. 91—68)

This invention relates to the manufacture and use of new compositions of matter suitable for serving as packing for fluid seals. More particularly it relates to the art of sealing moving parts of pumps or valves wherein the packing materials are required to resist the solvent action of organic chemicals such as acids, ketones, hydrocarbons, esters and alcohols under high pressure, and to retain these liquids without leakage.

10 The packing problem is indeed a very old one, and the most diverse compositions of matter have been described for serving the purpose. In general, the more common packing materials of the prior art are composed of fibrous substances impregnated with various lubricants. Such compositions may consist of leather or fibers of vegetable origin such as flax or hemp impregnated with fats or oils. In addition, graphite is frequently added to these fibrous grease-impregnated packing materials to give them better lubricating properties. Mineral fibers are also used, as in a packing consisting of asbestos yarn impregnated with paraffin or tallow. Another type of packing which has found extensive use consists of soft shredded metals impregnated with grease and graphite or both.

This invention has as an object certain improvements in compositions of matter suitable for use as packing.

30 The objects of my invention are accomplished by impregnating fibrous materials of vegetable, animal or mineral origin with high melting natural or synthetic waxes or wax-like bodies which are resistant to the solvent action of esters. 35 For example, I have made extensive tests of the solubilizing action of ethyl butyrate and other organic solvents on such waxes as beeswax, spermaceti, and hydrogenated castor oil. Of the above named materials the last is remarkably 40 resistant to the action of the solvents and constitutes an example of the material suitable for incorporation into the new compositions of matter described in this invention. It has been found that hydrogenated castor oil, in which the 45 unsaturation ordinarily present in castor oil has been satisfied either partially or completely through the addition of hydrogen, with the production of a body having the physical characteristics of a wax, possesses a remarkable resistance 50 to the action of such solvents as are commonly encountered.

In order to overcome the brittleness of some of these waxes or wax-like materials, I may add softeners thereto, said softeners likewise being

immune to the attack of the solvent. Preferred softeners are salts of the higher fatty acids, i. e., soaps, such salts being insoluble in organic solvents. Common soap in a dry condition has been found to be a suitable softener for hydrogenated 5 castor oil. In addition to the ingredients already named I may use solid lubricants such as graphite.

The following examples show how my invention may be carried out in practice:

10

## Example 1

Fifty grams of completely hydrogenated castor oil having a melting point of 80–85° C. was melted, 15 and 7.5 grams of graphite added. To this mixture there was added a section of asbestos yarn weighing about 10 grams. The melted oil was heated to 200° C., and triturated with the asbestos yarn for about 15 minutes after which the yarn was removed, drained, and allowed to cool. The 20 impregnated asbestos obtained under these conditions contained about 52% of the hydrogenated fat.

## Example 2

Two hundred twenty grams of hardened castor oil having a melting point of 75° C. was melted and heated to 200° C. At this temperature, there was added 25 grams of dry sodium stearate and 30 grams of flake graphite. Fifty grams of 30 shredded asbestos was triturated in the melted fat mixture at 200° C. for 10 minutes, removed, drained and allowed to cool, after which it was teased out in fine shreds.

## Example 3

One-eighth inch asbestos yarn was impregnated by passing it through a melted mass of hydrogenated castor oil having a melting point of 70° C.

35

## Example 4

Leather washers of a suitable size to fit into the stuffing box of a high pressure solvent pump were heated for five minutes at 110° C. in melted hydrogenated castor oil having a melting point of 45 84° C. Two or more of the treated washers were placed around the piston rod of the pump and forced down with a follower threaded into the stuffing box, until a durable leak-proof seal had been effected.

50

## Example 5

Shredded lead was impregnated with one-tenth of its weight of hydrogenated castor oil having a melting point of 75° C. and 1% of graphite.

55

**Example 6**

5 A mixture of asbestos and linen fibers were felted together in the presence of melted hydrogenated castor oil and rolled into sheets of suitable thickness for the cutting out of gaskets. This gasket material provides an effective seal when placed between sections of alcohol distillation columns and like equipment exposed to the solvent action of organic compounds.

**Example 7**

15 In carrying out the catalytic hydrogenation of ethyl butyrate a chemical proportioning pump having a 0.25" piston was employed to force the ester against 3000 lbs. of hydrogen pressure at the rate of 200 cc. per hour. Considerable difficulty was experienced in satisfactorily packing the pump under these conditions, and all available standard packing materials were tried.

20 Leather impregnated with neat's-foot oil, asbestos impregnated with paraffin, and a packing consisting of asbestos, stearin, and graphite were some of the materials that developed serious leaks within a few hours of operation.

25 As illustrating the advantages accruing from using the compositions of the present invention, under the same conditions of operation when the pump was packed with a composition comprising asbestos impregnated with hydrogenated castor oil and graphite prepared as described in Example 1, no leakage of the ester through the stuffing box was experienced until after a week's continuous operation.

**Example 8**

35 In another process liquid methyl alcohol was pumped against a pressure of only 200 lbs. per square inch, but leakage developed in half an hour when the pump was packed with a standard 40 prior art packing containing grease, graphite, and asbestos.

45 On the other hand, when asbestos impregnated with hydrogenated castor oil was employed as the pump packing and the process operated under the same conditions as before, no leakage had developed after 200 hours of operation.

50 In the above examples I have indicated one material which may serve as the waxy component of my new compositions, namely, castor oil which has been hydrogenated. The invention is not limited to this however, for any other wax or waxy material in the form of a single compound or a mixture having similar properties may be used instead. Such other waxy compound or 55 mixture used however will be a high melting derivative of a fatty acid, the melting point being preferably 70° C. or higher, since I have found that such materials in general possess the desired resistance to the action of organic solvents.

60 The fibrous component may be of vegetable, animal or mineral origin. For example, leather, silk or wool, or cotton, hemp, flax or jute fibers or fabrics may be used. Asbestos is, however, to be preferred but it may be used in conjunction 65 with any of the aforementioned fibers. In certain cases it may even be desirable to use a metallic fiber base, either alone or together with one or more of the fibers already mentioned. Graphite may or may not be included in the 70 composition depending on the exact use to which it is to be put. The exact method of impregnating the fibrous material with the waxy component may be varied within wide limits. The fiber base may be woven or braided into strands and later 75 impregnated by dipping into the melted wax

and graphite. Alternatively the elementary fibers may be incorporated into strands or fibers in the presence of or after mixing with the other components. The final compositions may be used in the form of rope, string or strands, or in molded forms such as rings, discs, or sheets.

5 The new compositions of matter described above are intended primarily for use in packing pumps and valves. They may also be used in other types of stuffing boxes such as are employed in gauge glasses, hydraulic lifts, and presses. The new packing materials are also well suited to use as gasket material. While they are admirably suited for use in the presence of organic liquids such as acids, ketones, hydrocarbons, esters and alcohols, they may also be used, of course, for packing against other fluids such as compressed air, oil, steam, water, and aqueous solutions.

10 Packing compositions such as have been described in the prior art are suitable for use at low pressures or in pumping or otherwise retaining liquids which do not have a solvent action on the packing, but owing to the rapid development of processes requiring the application of high pressures many of the older compositions are entirely 15 inadequate. The most extreme requirements are experienced in packing pumps to be used on organic solvent mixtures at high pressures, as in the high pressure dehydrogenation of ethanol or 20 the hydrogenation of organic acids, and esters, for example, in carrying out the process of U. S. Patent No. 1,708,460 and that described in my co-pending specification No. 445,224, filed April 17, 1930. No packing compositions of the prior 25 art have been found capable of enduring for long 30 the action of organic acids, and esters at pressures in excess of 100 atm. By use of the new materials described in this specification it is 35 now possible to pack the shafts of pumps in such 40 a manner that no leakage takes place over a long 45 period of continuous operation.

50 The above description and specific examples are to be taken as illustrative only. Any departure therefrom which conforms to the spirit of 45 the invention is intended to be included within the scope of the claims.

I claim:

1. A fluid-sealing material comprising a fibrous base impregnated with a hydrogenated castor 50 oil, said castor oil having been hydrogenated to such a degree as to produce a waxy material having a melting point of at least 70° C.

2. A fluid-sealing material comprising a fibrous base impregnated with a hydrogenated castor 55 oil, and with a softener for said hydrogenated castor oil consisting of a fatty acid soap.

3. A fluid-sealing material comprising a fibrous base impregnated with a mixture comprising a hydrogenated castor oil, and a solid lubricant, 60 said castor oil having been hydrogenated to such a degree as to produce a waxy material having a melting point of at least 70° C.

4. The method of making a fluid-sealing material which comprises passing a body of a fibrous base into a bath containing a molten hydrogenated castor oil, then removing the impregnated base from the bath, said castor oil having been hydrogenated to such a degree as to produce a waxy material having a melting point of at 65 70° C.

5. The method of sealing fluids which comprises applying to fluid leakage outlets a packing composition comprising a fibrous base impregnated with a hydrogenated castor oil, said 75

castor oil having been hydrogenated to such a degree as to produce a waxy material having a melting point of at least 70° C.

5. In a method of carrying out a catalytic reaction under high pressure wherein at least one of the reactants is an organic solvent, the step which comprises preventing leakage by packing fluid leakage outlets with a composition comprising a fibrous base impregnated with a hydrogenated castor oil, said castor oil having been hydrogenated to such a degree as to produce a waxy material having a melting point of at least 70° C.

10. The method of making a fluid-sealing material which comprises the steps of heating hydrogenated castor oil and a fatty acid soap to form a molten mixture and impregnating a fibrous base material with the molten mixture, said castor oil having been hydrogenated to such 15 a degree as to produce a waxy material having a melting point of at least 70° C.

20. The method of making a fluid-sealing material which comprises the steps of heating hy-

drogenated castor oil and an inert solid lubricant to form a molten mixture and impregnating a fibrous base material with the molten mixture, said castor oil having been hydrogenated to such a degree as to produce a waxy material having 5 a melting point of at least 70° C.

9. The method of making a fluid-sealing material which comprises the steps of heating hydrogenated castor oil, dry sodium soap, and graphite to form a molten mixture, triturating a fibrous 10 base material in the molten mixture to impregnate it with the material.

10. The method of making a fluid-sealing material which comprises the steps of heating to about 200° C. hydrogenated castor oil, adding 15 thereto dry sodium stearate and flaked graphite so as to obtain a mixture having approximately 10% sodium stearate and 12% graphite, triturating shredded asbestos in the molten mixture about 10 minutes, removing, draining, and allowing to cool the impregnated asbestos.

WILBUR A. LAZIER.